# EUROPEAN PATENT SPECIFICATION

(11) **EP 1 954 422 B1**
(45) Date of publication and mention of the grant of the patent: **08.12.2010**
(21) Application number: 06793177.4
(22) Date of filing: 04.09.2006
(51) Int. Cl.: B21F 45/22, B21F 45/16, B05D 7/20, B29C 47/02

(54) **USE OF A STEEL WIRE WITH A THICK POLYMER COATING AS BOOKBINDING WIRE**
VERWENDUNG EINES STAHLDRAHTES MIT DICKER POLYMERBESCHICHTUNG ALS BUCHBINDEDRAHT
UTILISATION D'UN FIL EN ACIER COMPORTANT UN REVETEMENT POLYMERIQUE EPAIS COMME SPIRALE DE RELIURE

(30) Priority: 22.11.2005 EP 05111048
(43) Date of publication of application: 13.08.2008
(73) Proprietor: NV Bekaert SA, 8550 Zwevegem (BE)
(72) Inventor: LEPLAE, Alain, B-8560 Moorsele (BE); POELMAN, Peter, B-9620 Velzele (BE); GROB, André, B-8510 Marke (BE)
(86) International application number: PCT/EP2006/065958
(87) International publication number: WO 2007/060040

(56) References cited:
- EP-A- 0 011 883
- WO-A-00/36177
- DE-A1- 2 104 271
- GB-A- 1 178 143

## Description

### Field of the Invention.

This invention relates to the use of a steel wire provided with a coating of an extrudable polymer as a bookbinding wire.

### Background of the Invention.

Steel wires provided with an extrudable polymer coating, such as polyvinylchloride, are generally known and are e.g. described in USA patent 4107370 and EP application 0011883.

USA patent 4107370 describes steel wires with thin polymer coatings, whereas EP application 0011883 describes in one example a steel wire with a thick polymer coating.

Until now, steel wires with a thin polymer coating are used as bookbinding wire (see e.g. WO-A-00/36 177, which forms the basis for the preamble of claim 1).

It is known that many mechanical properties of steel wires are seriously improved by increasing the diameter of the steel wires. However, a disadvantage thereof is that the weight of such steel wires with higher diameter is also seriously increased due to the high density of steel.

On the other hand, wires existing only of an extrudable polymer, i.e. without a steel core, also exist. They have the advantage of a lower weight and of a great degree of elasticity. For example, when these polymer wires take the form of a helix for use as bookbinding wire , these wires bounce back or rebound to the original form after being subjected to a transversal force. On the other hand, these polymer wires have various disadvantages. One disadvantage is their slow process of manufacturing, particularly when the final form is to be a helix. Another disadvantage relates to the above-mentioned high elasticity, which is not always an advantage. When used as a bookbinding wire in the form of a helix, the ends may be sharp and may injure the users. Bending these ends into a less dangerous form is not possible without heat treatment, having regard to the high degree of elasticity.

It is an object of the present invention to use a wire as bookbinding wire, whereby the above-mentioned disadvantages are taken away.

It is an object of the present invention to use as bookbinding wire, wires with a considerable reduction of weight without giving in on some critical parameters.

These objects are achieved by the use of a coated steel wire as a bookbinding wire as defined in claim 1.

According to the invention, thinner steel cores, provided with substantially thick coatings of an extrudable polymer, whereby the total diameter of the coated steel wire is substantially increased, are used as bookbinding wire. However, due to the lower density of the polymer compared with steel, the coated steel wire, used as bookbinding wire according to the invention, is of a low weight. The steel cores have usually a round cross-section.

The terms "extrudable polymer" refer to various types of thermoplastics, which are extrudable and comprise various polymers, such as polyvinylchloride, polyamide, polyester, polyurethane, polypropylene, ...Polyvinylchloride is advantageous from an economic point of view, since it is widely available and is of relatively low cost.

The coated steel wire, used as bookbinding wire according to the invention, is **characterised in that** the diameter of the steel wire is at least 0,2 mm, that the thickness of the coating is at least 50 % of the steel diameter and that the total diameter of the coated steel wire is lower than 3 mm.

A first advantage of the coated steel wire, used as a bookbinding wire according to the invention, is that the coated steel wire is substantially lighter than a steel wire with the same diameter.

A second advantage of the coated steel wire, used as a bookbinding wire according to the invention, is that the cost for manufacturing this coated steel wire is very acceptable thanks to the low cost price of some polymers, such as polyvinylchloride.

It has now been found surprisingly by carrying out a great number of tests, that the mechanical properties of such coated steel wires, used as bookbinding wires according to the invention, are highly improved.

The invention will now be described into more detail by means of some mechanical tests with reference to the accompanying drawing wherein:
- FIGURE 1 shows a transversal cross-section of a coated steel wire used according to the invention ;
- FIGURE 2 shows a schematic view of the compression test on a coil in the transversal direction ;
- FIGURE 3 illustrates the use of the wire as a book binding wire according to the invention;
- FIGURE 4 illustrates the use of wire as a paper clip.

The mechanical tests are carried out to compare two samples 1 and 2 with a sample 3 according to the prior art.

FIGURE 1 shows a transversal cross-section of samples 1 and 2 or a transversal cross-section of a coated steel wire 10. The coated steel wire 10 comprises a steel wire 12 and an outer coating 14 of polyvinylchloride (PVC). A primer or adhesion promoting layer may be present between the steel wire 12 and the outer coating (not shown).

Sample 1 consists of a drawn bright steel wire 12 of low carbon content (lower than 0,20 % by weight) with a diameter of 0,50 mm and a PVC-coating thickness of 0,50 mm or a coated steel wire 10 with a diameter of 1,50 mm. It means that the thickness of the PVC-coating is substantially 100 % of the steel wire diameter 12.

Sample 2 consists of a bright steel wire 12 of high carbon content (with a carbon content by weight above 0,25 % and lower than 1 %) with a diameter of 0,40 mm and a PVC-coating thickness of 0,525 mm or a coated steel wire 10 with a diameter of 1,45 mm. It means that the thickness of the PVC-coating 14 is substantially 130 % of the steel wire diameter 12.

Sample 3 consists of a bright steel wire 12 of low carbon content with a diameter of 0,80 mm and without any coating.

The cross-section of steel wire 12 of the 3 samples 1, 2 and 3 is in the proportion of 25 to 16 to 64.

A great number of coiled springs 16 is made from the samples 1, 2 and 3 for carrying out the mechanical tests. Such a coiled spring 16 can be used as a book binding wire.

The following tests are carried out by means of the formed coils or coiled springs of samples 1, 2 and 3.

### A) Hysteresistest in tensile (pulling) load in axial direction of the coils

In this test the coils or springs are loaded until a certain value (the upper reversal point) and then unloaded until the preload-value. The test conditions are :
- preload : lower reversal point : 2 Newton (N.)
- preload speed : 200 mm/min.
- 1 cycle
- upper reversal point : 6 N., 8 N., 10 N. and 12 N.
- cycle speed : 200 mm/min.
- grip to grip separation : 4 windings

The total deformation, the elastic deformation and the plastic deformation are measured. The following tables summarize the obtained results :

| **Total deformation** **(%)** | | **Sample** | | |
|---|---|---|---|---|
| | | 1 | 2 | 3 |
| Upper reversal point | 6 | 3.78 | 5.65 | 2.91 |
| | 8 | 7.03 | 8.30 | 5.60 |
| | 10 | 10.69 | 14.11 | 12.67 |
| | 12 | 19.61 | 19.58 | 26.29 |

| **Plastic deformation** **(%)** | | **Sample** | | |
|---|---|---|---|---|
| | | 1 | 2 | 3 |
| Upper reversal point | 6 | 0.86 | 0.68 | 0.61 |
| | 8 | 2.83 | 1.15 | 1.92 |
| | 10 | 5.29 | 4.22 | 8.00 |
| | 12 | 14.50 | 9.74 | 21.33 |

The elastic deformation is equal to the difference between the total deformation and the plastic deformation.

Each number of the tables is the mean value of at least three tests.

As can be seen from this hysteresis test, the sample 3 has a higher plastic and total deformation with higher upper reversal point values than the samples 1 and 2.notwithstanding its higher diameter of 0,80 mm compared with a diameter of 0,5 mm, respectively 0,4 mm of samples 1 and 2. This shows a serious improvement of the mechanical properties of samples 1 and 2 in comparison with sample 3 in this test.

### B) Compression test in transversal direction on the coiled springs until plastic deformation or bend.

Figure 2 shows how the coiled spring 16 is loaded (pressed) between two plates 18 until the spring is plastically deformed or bent.

| **Sample** | **Force at deformation or bend** **(N.)** |
|---|---|
| 1 | 167 |
| 2 | 168 |
| 3 | 143 |

Each obtained value is the mean value of at least three tests.

This test again shows a serious improvement of the mechanical properties of samples 1 and 2 compared with sample 3 notwithstanding its higher diameter of 0,8 mm.

Sample 2 shows substantially the same value as sample 1 notwithstanding its lower steel wire diameter (0,4 mm) and lower total diameter (1,45 mm). This is probably thanks to its thicker PVC-coating.

### C) Hysteresistest in compression in transversal direction on the coils, whereby plastic, elastic and total deformation are measured.

In this test, the coils or springs are loaded in compression in transversal direction (see figure 2) until a certain value (the upper reversal point) and then again unloaded until the preload-value is reached. The test conditions are :
- preload value : lower reversal point : 2 N.
- preload speed : 5 mm/min.
- 1 cycle
- cycle speed : 5 mm/min.
- grip to grip separation : 4 windings.

The following results are obtained :

| **Sample** | **Total deformation** **(%)** | **Elastic deformation** **(%)** | **Plastic deformation** **(%)** |
|---|---|---|---|
| 1 | 3.71 | 3.01 | 0.70 |
| 2 | 3.92 | 3.32 | 0.60 |
| 3 | 2.28 | 1.75 | 0.53 |

Each obtained value is the mean value of at least three tests.

This test again shows very acceptable deformation values, particularly for the plastic deformation for the samples 1 and 2 compared with sample 3.

Sample 2 shows a lower plastic deformation than sample 1 notwithstanding its lower steel wire diameter and lower total diameter. This is probably thanks to its thicker PVC-coating.

### D) Hysteresistest in compression load in axial direction of the springs, whereby plastic, elastic and total deformation are measured.

In this test, the coils or springs are loaded until a certain value (the upper reversal value) and then unloaded until the preload value. The test conditions are :
- preload : lower reversal point : 2 N.
- preload speed : 200 mm/min.
- 1 cycle
- upper reversal point : 8 N.
- cycle speed : 200 mm/min.
- grip to grip : 4 windings

The following results are obtained :

| **Sample** | **Total deformation** **(%)** | **Elastic deformation** **(%)** | **Plastic deformation** **(%)** |
|---|---|---|---|
| 1 | 5.91 | 2.72 | 3.19 |
| 2 | 9.06 | 2.54 | 6.52 |
| 3 | 4.90 | 2.56 | 2.34 |

Each obtained value is the mean value of at least three tests.

Here again, very acceptable values are obtained for samples 1 and 2.

### E) Bending of coated springs + measurement of degree of rebounding

Following samples are subjected to a bending test:
- prior art wire: 1.13 mm low-carbon steel core coated with PVC until final diameter of 1.50 mm;
- invention wire 1: 0.50 mm low-carbon steel core coated with PVC until final diameter of 1.50 mm;
- invention wire 2: 0.40 mm high-carbon steel core coated with PVC until final diameter of 1.45 mm

The various sample wires are formed into a spring and this spring is clamped in a Gressel apparatus. After clamping, the spring is bent over an angle of 135°. Thereafter, the spring is freed and the angle deformation is measured. It is hereby understood that a measured angle of 180° points to a 100% degree of rebounding. The table hereunder summarizes the results.

**Table**

| **Prior art sample** | **sample 1** | **sample 2** |
|---|---|---|
| 102° | 170° | 165° |
| 97° | 173° | 166° |
| 101° | 170° | 158° |
| 107° | 175° | 160° |
| 102° | | |
| 103° | | |

It is clear that the samples 1 and 2 exhibit a degree of rebounding, which approaches 100%, while the prior art sample exhibits a remaining deformation.

From the above-described tests and other tests, it is clear that the diameter of the steel wire 12 is at least 0,2 mm and that the thickness of the PVC-coating 14 is at least 50 % of the steel wire diameter.

A preferred embodiment of the coated steel wire 10 is characterized in that the thickness of the coating 14 is lower than 150 % of the steel wire diameter.

A further preferred embodiment of the coated steel wire 10 is characterized in that the diameter of the coated steel wire 10 is lower than 5 mm and preferably lower than 3 mm.

The polyvinylchloride resins forming the PVC-coating 14 are commercially available vinylchloride homopolymers, as well as copolymers containing at least 75 percent by weight of vinylchloride and up to about 25 percent by weight of one or more other polymerised comonomers.

The foregoing vinylchloride homopolymers and copolymers can be combined with stabilisers, plasticisers and pigments to obtain some typical known characteristics of the PVC-coating 14.

As an alternative embodiment the wire may have two layers of different polymers.

The wire is used, according to the invention, as book binding wire.

FIGURE 3 illustrates the inventive use as book binding wire. The invention wire is in the form of a spiral binding wire 10 to bind a book 20. As mentioned above and if no precautions are taken, both ends of the spiral binding wire 10 may injure the users. The advantage of the steel core inside the spiral binding wire 10 is that it can be plastically deformed without the need for a heat treatment. Hence, the spiral binding wire 10 advantageously has so-called coil loops 22 where the ends are bent back so that injuring of users is less likely.

FIGURE 4 illustrates the use of a wire as a paper clip 24.

## Claims

1. Use of a coated steel wire as a book binding wire, said steel wire comprising a coating of an extrudable polymer, wherein the diameter of the steel wire is at least 0,2 mm, and the total diameter of the coated steel wire is lower than 3 mm **characterised in that** the thickness of the coating is at least 50 % of the steel diameter.

2. Use of a steel wire according to claim 1, **characterised in that** the thickness of the coating is lower than 200 % of the steel wire diameter.

3. Use of a steel wire according to claim 1 or claim 2, **characterised in that** the steel wire is a low carbon steel wire with a carbon content below 0, 20 %.

4. Use of a steel wire according to claim 1 or claim 2, **characterised in that** the steel wire is a high carbon steel wire with a carbon content above 0,25 % and lower than 1 %.

## Patentansprüche

1. Anwendung eines beschichteten Stahldrahts als Buchbinderdraht, wobei der besagte Stahldraht eine Umhüllung aus einem stranggepressten Polymer aufweist, wobei der Durchmesser des Stahldrahtes mindestens 0,2 mm beträgt, und der Gesamtdurchmesser des beschichteten Stahldrahtes kleiner als 3 mm ist.

2. Anwendung eines Stahldrahtes nach Anspruch 1, **dadurch gekennzeichnet, dass** die Dicke der Umhüllung niedriger als 200% des Durchmessers des Stahldrahtes ist.

3. Anwendung eines Stahldrahtes nach Anspruch 1 oder Anspruch 2, **dadurch gekennzeichnet, dass** der Stahldraht ein weicher Stahldraht mit einem Kohlenstoffgehalt von unter 0,20% ist.

4. Anwendung eines Stahldrahtes nach Anspruch 1 oder Anspruch 2, **dadurch gekennzeichnet, dass** der Stahldraht ein harter Stahldraht mit einem Kohlenstoffgehalt von über 0,25% und unter 1% ist.

## Revendications

1. Utilisation, en tant que spirale de reliure, d'un fil en acier comportant un revêtement, ledit fil en acier comprenant un revêtement en un polymère que l'on peut extruder, où le diamètre du fil en acier est d'au moins 0,2 mm et où le diamètre total du fil en acier recouvert est inférieur à 3 mm, **caractérisé en ce que** l'épaisseur du revêtement est au minimum égale à 50 % du diamètre de l'acier.

2. Utilisation d'un fil en acier selon la revendication 1 **caractérisé en ce que** l'épaisseur du revêtement est inférieure à 200 % du diamètre du fil en acier.

3. Utilisation d'un fil en acier selon la revendication 1 ou la revendication 2, **caractérisé en ce que** le fil en acier est un fil en acier à faible taux de carbone avec une teneur en carbone inférieure à 0,20 %.

4. Utilisation d'un fil en acier selon la revendication 1 ou la revendication 2, **caractérisée en ce que** le fil en acier est un fil en acier à taux de carbone élevé avec une teneur en carbone supérieure à 0,25 % et inférieure à 1 %.
